

March 11, 1952

R. J. LEE ET AL

2,588,639

PRODUCTION OF DRYING OILS BY HF-HYDROCARBON PROCESSING

Filed May 4, 1948



INVENTORS  
 Robert J. Lee  
 Paul D. May  
 BY Donald E. Payne  
 ATTORNEY

## UNITED STATES PATENT OFFICE

2,588,639

PRODUCTION OF DRYING OILS BY  
HF-HYDROCARBON PROCESSING

Robert J. Lee, La Marque, and Paul D. May, Galveston, Tex., assignors to Pan American Refining Corporation, Texas City, Tex., a corporation of Delaware

Application May 4, 1948, Serial No. 24,958

5 Claims. (Cl. 260—666)

1

This invention relates to the production of drying oils and other olefinic hydrocarbons by processing high boiling, non-aromatic hydrocarbons with hydrogen fluoride and it pertains more particularly to improved methods and means for obtaining maximum yields of high quality drying oils from dearomatized gas oil and for producing and recovering said drying oils with a minimum consumption or loss of hydrogen fluoride (herein referred to as HF).

It is known that drying oils can be produced by neutralizing or hydrolyzing certain HF-hydrocarbon complexes produced in hydrocarbon refining processes wherein HF is employed as the refining or treating agent. Heretofore such processes have lacked commercial feasibility because when HF complexes were neutralized the HF formed a salt with the neutralizing agent and when it was hydrolyzed with water it formed an aqueous solution from which anhydrous HF could not be obtained by commercially feasible methods (about .5 to .75 lb. HF was lost per pound of drying oil produced). An object of this invention is to provide a method and means for hydrolyzing HF-hydrocarbon complexes which method will enable recovery of substantially anhydrous HF by simple distillation and which will thereby substantially avoid any loss of HF by aqueous dilution or salt formation. An important object is to avoid or at least to minimize degradation, cracking, saturation or other undesirable reactions in the recovery step.

Another object is to provide a method for varying the yield and viscosity of the recovered drying oil. A subsidiary object is to provide a method for increasing the yield of viscous drying oil while decreasing the yield of low viscosity low molecular weight poly-olefin fractions. Another object is to produce a finished oil of good color and high viscosity without requiring further distillation of the recovered product for removal of undesirable fractions. A further object is to provide a means for controlling the degree of "bodying" of the recovered oil, without any substantial loss in unsaturation. A still further object is to accomplish the above objectives without interposing any additional processing steps for recovering the poly-olefinic oil, and while simultaneously facilitating the recovering of HF.

Another object of the invention is to provide an improved method and means for producing drying oils from hydrocarbon charging stocks such for example as ordinary gas oils available in the petroleum industry. A further object is to provide a drying oil of improved characteristics, with exceptionally high unsaturation (iodine number), high degree of conjugation, good color and high blending value as an agent in coating compositions and/or for the production of resins, plastics, and the like. A further object is to provide a

2

process, and operating conditions therefor, which will produce such drying oils in large yields while at the same time producing valuable by-product materials. Another object is to provide a relatively simple and inexpensive process for converting hydrocarbons which are higher boiling than gasoline into more valuable hydrocarbons such as drying oils and other olefinic hydrocarbons as well as substantially saturated hydrocarbons particularly of the motor fuel boiling range. Other objects will be apparent as the detailed description of the invention proceeds.

In practicing the invention a preferred charging stock is a gas oil which has been dearomatized by treatment with concentrated sulfuric acid. Many charging stock materials such, for example, as olefin polymers, alkylates, and hydrocarbons produced by carbon monoxide-hydrogen synthesis may contain no aromatic hydrocarbons and hence may require no dearomatization step. Relatively pure paraffinic hydrocarbons such as cetane and paraffin waxes may be employed but they give a less desirable product distribution and they are not as commercially attractive as the less valuable gas oils. The dearomatization may of course be effected by other means than treatment with sulfuric acid; the aromatics may be removed by use of known selective solvents but for best results it is important that the aromatic content of the charge be substantially eliminated, i. e. that the aromatic content should not materially exceed about 5% and preferably not more than 1%.

The HF treatment of the dearomatized gas oil or other charging stock may be effected at a temperature in the range of about 250 to 450° F., preferably about 300 to 350° F. under a pressure sufficient to maintain liquid phase conditions and with a time of contact which may range from a few minutes to several hours depending upon temperature and intimacy of said contact, excellent results having been obtained with contact times of the order of about 5 to 30, e. g. about 20 minutes. The HF-to-oil ratio may vary from about 2:1 to about 5:1 or more but is preferably in the range of about 1:1 to 2:1.

The products of the HF treatment are preferably cooled and separated into an HF phase containing soluble unsaturated hydrocarbons and an insoluble oil phase which consists essentially of saturated hydrocarbons and contains only a small amount of dissolved HF. The oil phase is stripped for removing HF and fractionated to produce motor fuel along with lighter and heavier fractions.

The HF phase separated from the product of the treating step is subjected to a partial stripping operation under carefully controlled conditions to remove most of the HF from an HF complex without decomposing or degrading said

complex. This can usually be accomplished at temperatures below about 250° F. and in most cases at temperatures in the range of about 100 to 200° F.; it may be accomplished by the use of an inert stripping gas or by heating. It is important that at least one and preferably one and one-half to two mols of HF should be left in the stripped residue for each "mol of double bonds" present therein; for practical purposes this means that the stripped residue should contain at least about 30% HF and preferably about 35 to 50% HF. One "mol of double bonds" as expressed herein represents an average of one ethylenic linkage per molecule of oil. By this terminology, therefore, one mol of a polyolefinic oil containing four ethylenic linkages per molecule would be equivalent to "four mols of double bonds." In other words, the stripping must leave about 1 to 2 molecules of HF per double bond in the hydrocarbon component of the hydrogen fluoride-hydrocarbon complex. If attempts are made to recover all of the HF by stripping or distillation, even at 100-125° F., the residue oil is degraded to dark tarry products of low degree of unsaturation.

The stripped complex which contains at least about 1 to 2 molecules of HF per double bond in the hydrocarbon component (i. e. the hydrocarbon product finally produced) is then hydrolyzed with an aqueous HF solution containing about 1 part to 3 parts of HF weight to 2 parts of water. The HF component of the hydrolyzing mixture does not interfere with effective hydrolysis and in fact appears to exert a beneficial effect in absorbing heat of hydrolysis. It should be noted that the aqueous HF is not employed in this case simply to remove free HF from a simple solution thereof, it is used to effect actual hydrolysis of a complex. The hydrolysis may be effected in a jacketed hydrolyzing vessel provided with a stirrer and sufficient hydrolyzing agent should be employed so that after subsequent separation the aqueous layer will contain at least one part of water to six parts of HF and preferably about 1 part of water to 1½ parts of HF.

The hydrolysis may be effected in a plurality of stages either with or without countercurrent contacting and preferably with cooling between stages. If sufficient intimacy of contact and adequate temperature control is provided the hydrolysis may be effected in a countercurrent tower. It is preferred that the temperature of hydrolysis be in the range of 30 to 200° F. during initial contacting. The hydrolyzed complex is thus substantially freed from HF, i. e. it contains less than about .2 to .3% HF by weight. Any residual HF is preferably removed from the hydrolyzed product by intimate contact with alkaline solution such as caustic ammonia, lime slurry, etc. The neutralized product may then be distilled with inert gas, steam or under vacuum to remove any low boiling components therefrom and to produce drying oils either as overhead or as undistilled fractions of desired molecular weight. The drying oils thus produced have remarkably high iodine numbers which usually range from about 400 to 500, they are usually characterized by 4 to 8 double bonds per molecule (about one pair in conjugated position) and they have surprisingly good color. A typical drying oil before distillation may have an average molecular weight of about 390, a viscosity of Z-2 Gardner at 25° C., an iodine number of about 440, an ASTM color of about 6-7 and a maleic anhydride value of about 165. In this connec-

tion, iodine number is understood to mean centigrams of iodine per gram of sample as determined by the Wijs' iodine monochloride procedure using ½ hour reaction time and 200% excess reagent. Maleic anhydride value (MAV) represents the milligrams of maleic anhydride which will react with one gram of sample (also referred to as the diene number) and is a measure of the amount of conjugated olefinic double bonds in the samples.

If the stripped complex is hydrolyzed with a carefully controlled amount of hydrolyzing agent such that the final weight ratio of HF to water in the aqueous layer is above about 1.2 (55 parts HF and 45 parts of water), the separated olefinic oil will be of considerably higher viscosity, (e. g. Z Gardner or higher) and will contain substantially no low boiling compounds. If the final ratio of HF to water in the aqueous phase is lower than about 0.8 (45 parts HF:55 parts water), the separated total olefinic oil after hydrolysis will be relatively non-viscous (e. g., less than L Gardner), and will contain 15-35% of low boiling fractions having a viscosity of less than A Gardner which are unsuitable for use as drying oils. If the stripped complex is hydrolyzed with an alkaline reagent such as ammonia or caustic solution, the separated total olefinic oil will have a Gardner viscosity of less than A and will contain 25-45% of low boiling fractions.

The aqueous layer from the hydrolysis step which may now contain about 0.8 to 1.2 parts of HF per one part of water by weight is subjected to a partial distillation step under conditions to remove substantially anhydrous HF overhead. However, if the first hydrolyzing operation is conducted so that the weight ratio of HF to water in the aqueous layer exceeds 1.2, said aqueous layer should be subjected to a second hydrolyzing step before distillation, in order to reduce the HF to water ratio in the aqueous layer to a value of 1.0-1.2. This is important since aqueous HF containing more than about 1.2 parts by weight of HF per part water will retain a considerable amount of olefinic oil in solution. The distillation of the aqueous HF solution is carefully controlled to distill substantially anhydrous HF overhead, thereby leaving about 1 part of HF per 1.5 parts of water in the aqueous solution which is withdrawn from this operation and again utilized in the hydrolysis step. Thus in normal operation no water is added to the system and no aqueous HF has to be withdrawn therefrom. The water component simply goes round and round in the hydrolyzing cycle and the HF removed from the complex is thus recovered in substantially anhydrous condition for reuse in the treating step.

The invention will be more clearly understood from the following detailed description read in conjunction with the accompanying drawings in which:

Figure 1 is a schematic flow diagram illustrating a commercial plant for practicing the invention, and

Figure 2 is a hydrolysis system utilizable in the system of Figure 1.

Before describing the operation illustrated in the drawings, data will be presented to show the importance and significance of operating conditions. A preferred charging stock is dearomatized gas oil. The following table sets forth data obtained by treating various charging stocks with a 2:1 HF/oil weight ratio at a temperature of about 330° F. for a contact time of about 20 min-

utes in an autoclave provided with a motor-driven propeller-type agitator. In these runs, at the end of the reaction period, the reaction mixture was allowed to settle while cooling to room temperature. The lower HF phase was then withdrawn from the bomb through a Saran tube into a neutralizing mixture of aqueous ammonia and cracked ice. The transparent Saran tubing served as a means of noting when the interface between the acid and the hydrocarbon phases had been reached. The ammonium-fluoride solution was allowed to settle and the poly-olefinic oil was decanted from the solution. The hydrocarbon phase from the reactor was neutralized in a similar fashion and collected separately.

#### Effect of charge stocks

| Charge Stock             | C <sub>15</sub><br>Branched<br>Olefin <sup>1</sup> | C <sub>16</sub><br>Normal<br>Olefin <sup>2</sup> | C <sub>15</sub><br>Branched<br>Paraffin <sup>3</sup> | C <sub>16</sub><br>Normal<br>Paraffin <sup>4</sup> |
|--------------------------|----------------------------------------------------|--------------------------------------------------|------------------------------------------------------|----------------------------------------------------|
| Vol. per cent Conversion | 93-100                                             | (100)                                            | 26.1                                                 | 43.3                                               |
| Yield of Unsat'd. Oil    | 38.2                                               | 28.8                                             | 8.9                                                  | 15.2                                               |
| Iodine No.               | 440                                                | 467                                              | 503                                                  | 475                                                |
| Refractive Index         | 1.526                                              | 1.507                                            | 1.502                                                | 1.498                                              |
| Molecular Weight         | 212                                                | 205                                              | 205                                                  | 213                                                |

| Charge Stock             | C <sub>8</sub> Branched<br>2,2,4-Tri-<br>methyl pentane | Dearomatized Gas Oils |                              |
|--------------------------|---------------------------------------------------------|-----------------------|------------------------------|
|                          |                                                         | Paraffin <sup>5</sup> | Naph-<br>thenic <sup>6</sup> |
| Vol. per cent Conversion | 95.7                                                    | 58.7                  | 65                           |
| Yield of Unsat'd. Oil    | 19.5                                                    | 24.3                  | 22.3                         |
| Iodine No.               | 506                                                     | 475                   | 481                          |
| Refractive Index         | 1.4910                                                  | 1.517                 | 1.503                        |
| Molecular Weight         | 185                                                     | 225                   | 201-229                      |

<sup>1</sup> Tetra isobutylene fraction recovered from isobutylene polymer produced by H<sub>2</sub>SO<sub>4</sub> polymerization.

<sup>2</sup> Normal-hexadecene, 95% purity.

<sup>3</sup> Product from complete hydrogenation of (1).

<sup>4</sup> Cetane, 95% purity.

<sup>5</sup> East Texas gas oil (400°-650° F. boiling range dearomatized by exhaustive sulfuric acid treating to a reduced aromatic content of less than 1%).

<sup>6</sup> Hastings gas oil (400-650° F. boiling range, dearomatized by exhaustive sulfuric acid treating to a reduced aromatic content of less than 1%).

When consideration is given to percent conversion, unsaturated oil yield in conversion products and iodine number of unsaturated oil, it will be noted that the dearomatized gas oils provide the best charging stocks particularly when their cost is compared with that of other charging stocks. The effect of dearomatization is shown by comparative tests on a virgin East Texas gas oil as compared with the same gas oil after de-

5  
6 aromatization by repeated treatment with sulfuric acid. Employing the same treating conditions (2:1 HF-oil weight ratio, 330° F. and 20 minutes contact time, hydrolysis with aqueous ammonia) the following comparative data were obtained:

|    | Charge Stock                                     | Virgin<br>Gas Oil | Dearo-<br>mated<br>Gas Oil |
|----|--------------------------------------------------|-------------------|----------------------------|
| 10 | Aromatics                                        | 17.0              | <1                         |
|    | Volume Per Cent Conversion                       | 40.5              | 59                         |
|    | Yields (Vol. Per Cent on CHG):                   |                   |                            |
|    | Dry Gas                                          | .4                | 1.2                        |
|    | Isobutane                                        | 4.3               | 12.0                       |
|    | Normal Butane                                    | .1                | 1.0                        |
|    | Butenes                                          | .0                | .1                         |
|    | Pentanes                                         | 2.2               | 6.5                        |
| 15 | Pentenes                                         | .4                | 1.0                        |
|    | C <sub>6</sub> -205° C.                          | 15.1              | 12.9                       |
|    | Total                                            | 22.5              | 34.7                       |
|    | Recycle gas oil                                  | 59.5              | 40.7                       |
| 20 | HF soluble product:                              |                   |                            |
|    | Below 205° C.                                    | 1.9               | 4.0                        |
|    | Gas oil range                                    | 5.6               | 11.2                       |
|    | Heavier than gas oil                             | 9.2               | 8.1                        |
|    | Total                                            | 16.7              | 23.3                       |
|    | Properties of HF Soluble Oil:                    |                   |                            |
|    | Iodine Number (Wijs, 1/2 hr.)                    | 297               | 475                        |
|    | Specific Gravity (60°/60° F.)                    | .9786             | .9059                      |
|    | Refractive Index (n <sub>D</sub> <sup>20</sup> ) |                   | 1.505                      |
| 25 | Gardner Viscosity at 25° C.                      |                   | 1 A-4                      |

<sup>1</sup> Approximately 6 centistokes.

The effect of aromatics on the nature and extent of the conversion is strikingly illustrated in the above table. With respect to the HF-soluble products, the pronounced difference in proportions and particularly in degree of unsaturation is shown by the following comparative data on respective HF-soluble products after neutralization to remove final traces of HF and after removing C5 and lighter hydrocarbons.

#### HF-Soluble products from

| Fraction—Approx. Boiling Range | East Texas Gas Oil       |               | Dearomatized Gas Oil |               |     |
|--------------------------------|--------------------------|---------------|----------------------|---------------|-----|
|                                | Per Cent                 | Iodine Number | Per Cent             | Iodine Number |     |
| 45                             | IBP to 110° C. at 50 mm. | 12            | 147                  | 17            | 525 |
|                                | 60°-104° C. at 1 mm.     | 33            | 315                  | 48            | 485 |
|                                | 154-200° C. at 1 mm.     | 27            | 255                  | 12            | 445 |
|                                | Bottoms (Tar)            | 28            | 181                  | 23            | 348 |
|                                | Total Oil                | 100           | 297                  | 100           | 475 |

50 A more detailed analysis of the HF-soluble product from the treating of virgin East Texas gas oil is as follows:

| Cut No. | Vol. per cent on Chg. | Ovhd. Temp. at mm. Hg. | Estimated Ovhd. Temp. At 760 mm. °F. | Iodine Number | 25 nD | Sp. Gr. At 25° C. | McL. Wt. |
|---------|-----------------------|------------------------|--------------------------------------|---------------|-------|-------------------|----------|
|---------|-----------------------|------------------------|--------------------------------------|---------------|-------|-------------------|----------|

#### GASOLINE RANGE MATERIAL

|     |        |     |     |     |      |        |       |
|-----|--------|-----|-----|-----|------|--------|-------|
| IBP |        | 70  | 765 | 158 |      |        |       |
| 1   | 1.0    | 100 | 765 | 212 | .48  | 1.4090 | .7258 |
| 2   | 10.7   | 110 | 46  | 370 | .157 | 1.4650 | .8267 |
|     | (11.7) |     |     |     |      |        | 133   |

#### GAS OIL RANGE MATERIAL

|   |        |     |   |     |     |        |       |     |
|---|--------|-----|---|-----|-----|--------|-------|-----|
| 3 | 16.7   | 105 | 1 | 555 | 336 | 1.5135 | .9086 | 177 |
| 4 | 16.7   | 136 | 1 | 620 | 293 | 1.5350 | .9384 | 197 |
|   | (33.4) |     |   |     |     |        |       |     |

#### HEAVIER THAN G. O. RANGE MATERIAL

|                |        |     |   |     |     |        |        |     |
|----------------|--------|-----|---|-----|-----|--------|--------|-----|
| 5              | 16.7   | 185 | 1 | 725 | 237 | 1.5550 | .9716  | 230 |
| 6              | 10.3   | 217 | 1 | 800 | 273 | 1.5783 | .9976  | 233 |
| Bottoms        | 27.9   |     |   |     | 181 |        | 1.0928 | 467 |
|                | (54.9) |     |   |     |     |        |        |     |
| Total Material |        |     |   |     | 297 |        | .9632  |     |

7 For comparison, properties of the HF-soluble product obtained from the HF treating of de-aromatized gas oil are as follows:

to-fore obtainable from petroleum, but the striking difference between such drying oil and the

| Cut No.                           | Vol.<br>per cent<br>on Chg. | Ovhd.<br>°C. | Temp. at<br>mm. Hg | Estimated<br>Ovhd. Temp.<br>At 760 mm.<br>°F. | Iodine<br>Number | 25<br>nD | Sp. Gr.<br>At 25° C. | Mol.<br>Wt. |
|-----------------------------------|-----------------------------|--------------|--------------------|-----------------------------------------------|------------------|----------|----------------------|-------------|
| GASOLINE RANGE MATERIAL           |                             |              |                    |                                               |                  |          |                      |             |
| IBP.....                          |                             | 48.5         | 775                | 119                                           | 33               | 1.3860   | .6815                | 102         |
| 1.....                            | 2.6                         | 100          | 775                | 212                                           | 613              | 1.4665   | .8371                | 132         |
| 2.....                            | 14.6                        | 110          | 50                 | 385                                           |                  |          |                      |             |
|                                   | (17.2)                      |              |                    |                                               |                  |          |                      |             |
| GAS OIL RANGE MATERIAL            |                             |              |                    |                                               |                  |          |                      |             |
| 3.....                            | 16.0                        | 106.5        | 0.9                | 560                                           | 510              | 1.5001   | .9049                | 186         |
| 4.....                            | 16.0                        | 125          | 0.9                | 595                                           | 500              | 1.5081   | .9195                | 220         |
| 5.....                            | 16.0                        | 154          | 0.8                | 600                                           | 1.460            | 1.5165   | .9354                | 256         |
|                                   | (48.0)                      |              |                    |                                               |                  |          |                      |             |
| HEAVIER THAN G. O. RANGE MATERIAL |                             |              |                    |                                               |                  |          |                      |             |
| 6.....                            | 11.3                        | 185          | 1.2                | 720                                           | 2445             | 1.5260   | .9508                | 279         |
| Bottoms.....                      | 23.5                        |              |                    |                                               | 348              |          |                      | 379         |
| Total Material.....               | (34.8)                      |              |                    |                                               | 475              |          | .9059                |             |

<sup>1</sup> Gardner viscosity at 25° C. = A (ca. 50 cs or 230 SSU at 25° C.)

<sup>2</sup> Gardner viscosity at 25° C. = L (ca. 300 cs or 1460 SSU at 25° C.)

The above data show that there is a striking difference in properties of HF-soluble products produced when the gas oil is initially dearomatized. Aromatics apparently have a deleterious effect and they apparently produce HF-soluble condensation and alkylation products which dilute and degrade the polyolefin products and thereby decrease their value as drying oils.

In addition to the above properties of HF-soluble products produced from dearomatized gas oil it is noteworthy that such products possess a high maleic anhydride value (MAV). For example, cut No. 2 had an MAV of 625 which with its iodine number of 613, molecular weight of 132, and refractive index of 1.4665 indicates a mixture of tri and tetra olefins (3.2 double bonds per mol) which are largely conjugated in structure; i. e. at least 85% of the molecules have one pair of conjugated double bonds. This was qualitatively confirmed by ultra violet spectrophotometric observation. A blend of cuts 4, 5 and 6 showed an MAV of 302, an iodine number of 475, a refractive index of 1.517 and a molecular weight of 250; this indicates that the material is composed of polyolefins containing approximately 4 or more double bonds per molecule and that about 75 to 80% of the material contains one pair of double bonds in conjugation. This is a very unusual combination of properties.

The colors of the vacuum distillate fractions were good varying from 1-1½ for the lower boiling components to 3½-5 ASTM for the high boiling products.

For use in the drying oil and/or resin field, cuts 4, 5 and 6 (which represent approximately 43% of the total HF-soluble product) possess the requisite low volatility and adequate body (viscosity) to meet commercial requirements. Each of these fractions air dry readily and, a composite sample produced a film corresponding to a "polymer" drying oil produced by contacting unrefined cracked gasoline vapors with an adsorbent clay under conditions for removing and polymerizing diolefins. Such clay polymer is believed to represent the best drying oils here-

5 drying oil of this invention is shown by the following tabulated properties:

|                                              | Drying oil<br>from HF<br>treating of<br>dearom.<br>gas oil <sup>1</sup> | Drying Oil<br>from Clay<br>Polymer |
|----------------------------------------------|-------------------------------------------------------------------------|------------------------------------|
| Boiling Range °C. at 1 mm. Hg.....           | 106-185                                                                 | 104-225                            |
| Refractive Index at 25° C.....               | 1.5178                                                                  | 1.5365                             |
| Specific Dispersion ( $n_F/n_C$ ).....       | 150                                                                     | 170                                |
| Specific Gravity at 25° C.....               | 0.9274                                                                  | 0.969                              |
| Iodine Number.....                           | 439                                                                     | 189                                |
| M. A. V.....                                 | 302                                                                     | 27                                 |
| 40 Per Cent Conjugation (from M. A. V.)..... | 77                                                                      | 7                                  |
| Approximate Mol. Weight.....                 | 250                                                                     | 290                                |
| Viscosity at 100° F.:                        |                                                                         |                                    |
| Centistokes.....                             | 17.28                                                                   | 41.7                               |
| Saybolt Universal Sec.....                   | 86                                                                      | 194                                |
| Color:                                       |                                                                         |                                    |
| Gardner.....                                 | 13                                                                      | 15                                 |
| ASTM.....                                    | 4+                                                                      | 5                                  |
| 45 Drying Time:                              |                                                                         |                                    |
| (Set to touch)-Hrs. <sup>2</sup> .....       | 1½-2½                                                                   | 1½-2½                              |
| (Tack-free)-Hrs.....                         | 6-8                                                                     | 6-8                                |

<sup>1</sup> Composite of cuts 4, 5 and 6.

<sup>2</sup> With 0.5% lead naphthenate and 0.05% cobalt naphthenate driers.

50 Referring now to the effect of process variables in producing the polyolefin or drying oil materials, the most important are HF/oil ratio, contact time (assuming intimate mixing) and temperature. As the HF/oil weight ratio is increased from about .25:1 to about 3:1 there is a gradual increase in product iodine number and a substantial increase in yield. HF/oil ratios below about 1:1 are usually undesirable not only because of limited yield and lower product unsaturation but because of limited physical capacity of the available HF to dissolve the polyolefinic material. The preferred HF/oil ratio is about 1:1 to 2:1 and it is usually uneconomical to employ a greater ratio than 5:1. The properties of the drying oil are not substantially affected by changes in the HF/oil ratio.

55 The required contact time is dependent on temperature and intimacy of contact; higher temperatures make possible the use of shorter contact times. With an HF/oil ratio of 2 (i. e. 2:1) and a 20 minute contact time, a yield of about 12% is obtained at 265° F. (iodine number 461) while a yield of about 22% is obtained at about 300° F. (iodine number about 510). Adequate conversion at lower temperatures may re-

quire a contact time of an hour or more. At temperatures of the order of 400° F. the contact time for equivalent conversion may be of the order of about 3-5 minutes. Thus the time of contact may vary from about a minute to an hour or more depending upon the temperature employed but at preferred temperatures such contacting time is in the range of about 5 to 30 minutes, e. g. about 15 to 20 minutes. The preferred temperature is in the range of about 300 to 400° F. The iodine number has been observed to decrease with excessively long contact times, said decrease being accompanied by an increase in molecular weight and specific gravity.

It should be pointed out that in all of the

5 The desirability of leaving at least one and preferably one and one half to two molecules of HF per double bond in the poly-olefinic oil present in the partially stripped complex is thus demonstrated.

10 Using partially stripped complex containing approximately 40% HF, a series of experiments were conducted in which the stripped complex was hydrolyzed by slowly pouring the partially stripped complex into a water cooled jacketed copper vessel equipped with an agitator and containing varying amounts of water. The following table shows the concentration of HF in the aqueous HF layer together with the properties of the recovered oils.

| Run No. | HF in aqueous layer (weight per cent) | MAV | Sp. gr. of Rec. Oil (60° F.) | I <sub>2</sub> No. of Rec. Oil | M.W. of Rec. Oil | Viscosity at 25° C. |         |
|---------|---------------------------------------|-----|------------------------------|--------------------------------|------------------|---------------------|---------|
|         |                                       |     |                              |                                |                  | (Gardner)           | (C. S.) |
| Ammonia | Neut. Oil                             | 362 | .918                         | 486                            | 225              |                     |         |
| A       | 22.6                                  | 362 | .9165                        | 495                            | 233              | A                   | 6-25    |
| B       | 26.5                                  | 362 | .9190                        | 490                            | 233              | A+                  | 50-65   |
| C       | 43.0                                  | 362 | .9340                        | 470                            | 295              | A+                  | 50-65   |
| D       | 58.0                                  | 164 | .9434                        | 432                            | 391              | E                   | 125     |
|         |                                       |     |                              |                                |                  | Z-6                 | 14,800  |

above examples, the HF phase from the treating step was withdrawn and hydrolyzed in aqueous ammonia containing cracked ice. The recovered olefinic oil is of relatively low viscosity and contains a substantial amount of relatively non-viscous light fractions. By effecting the hydrolysis under carefully controlled conditions with aqueous HF, the viscosity of the recovered oil is increased to an unusual degree and the proportion of low viscosity light fractions is reduced considerably or substantially eliminated.

Prior to hydrolysis, the HF phase is partially stripped to remove most of the HF from the HF complex. The importance of leaving at least one and preferably one and one half to two molecules of HF per double bond present in the oil is illustrated by the following run made on HF phase material produced by HF treating of dearomatized naphthenic gas oil substantially as hereinabove described. The HF phase material was charged to a continuous type stripping column packed with carbon Raschig Rings. The stripping was conducted in countercurrent fashion at stripping rates equivalent in most cases to approximately 1 cubic foot of natural gas per liter of HF phase per minute. By varying the heat input to the nichrome wire wrapped in sections around the stripping tower, various degrees of removal of HF were attained as shown in the summary table below. The relationship between the iodine number of the stripped and recovered oil (after final ammonia neutralization) and the HF content of the residual stripped oil (before neutralization) is especially noteworthy.

30 This shows the marked effect of controlling the HF concentration during the hydrolyzing step on the viscosity, MW, and other properties of the recovered oil. (MW signifies molecular weight-Menzies-Wright.)

35 Referring now to the drawing, a dearomatized gas oil (or other substantially nonaromatic high boiling hydrocarbon charge) is introduced by line 10 through heater 11 to reactor 12 together with HF introduced through line 13, about 2 parts by weight of HF in this case being introduced per part of oil charge. The reactor may be a batch type or continuous reactor of any known type which will give sufficient intimacy of contact for the required period of time and 40 it is illustrated as a cylindrical vessel provided with a mechanical stirrer 14 driven by motor 15. In the reactor conversion is effected at a temperature of about 330° F. with a contact time of about 20 minutes under a pressure sufficient to maintain liquid phase conditions, e. g. about 800 to 1500 p. s. i. The charge should of course be dry when it is introduced into the system and conventional drying towers may be employed when necessary. The reactor and other elements 45 must of course be fabricated from or lined with metals, alloys or compositions which are resistant to hydrogen fluoride corrosion and may for example be of Monel construction. The reactor may consist of a tank provided with a pump-circulated emulsion stream such as employed in conventional sulfuric acid alkylation operations. The intimate mixing in the reactor 50 may be obtained by the use of rotating shear discs adjacent to stationary plates. Since no in-

| Run No. | Approx. Stripping Temp. | Composition of Residual Stripped Oil |              |                                                | I <sub>2</sub> No. of Neutralized Oil | Sp. Gr. |
|---------|-------------------------|--------------------------------------|--------------|------------------------------------------------|---------------------------------------|---------|
|         |                         | Weight Per Cent of HF                | Per Cent Oil | Moles HF per Mole of Double Bonds <sup>1</sup> |                                       |         |
| 1       | 197                     | 0.5                                  | 99.5         | 0.1                                            | 269                                   | 0.9642  |
| 2       | 120                     | 10                                   | 90           | 0.33                                           | 340                                   | 0.9553  |
| 3       | 82                      | 20.3                                 | 79.7         | 0.68                                           | 408                                   | 0.944   |
| 4       | 79                      | 27.3                                 | 62.7         | 1.57                                           | 425                                   | 0.932   |
| 5       | 236                     | 41.9                                 | 58.1         | 1.92                                           | 454                                   | 0.929   |
| 6       | 81                      | 45.1                                 | 54.9         | 2.22                                           | 448                                   | 0.955   |
| (1)     |                         |                                      |              |                                                | 486                                   | 0.918   |

<sup>1</sup> Calculated on the basis of 475 I<sub>2</sub> No., 225 mol. wt. and 4.2 (=)/mole in all cases.

<sup>2</sup> Oil recovered by neutralization of total sample.

vention is claimed in the reactor per se it requires no further description.

The reaction mixture is passed through a cooler 16 before being introduced from line 17 to product separator 18. The separator or settler 18 may be operated at substantially reaction pressure but at a temperature below about 250° F. and preferably in the range of about 80 to 180° F. The insoluble saturated oil fraction flows over baffle 19 and is withdrawn through line 20 to stripper 21 which is provided with conventional heating means 22 at its base. Substantially all of the HF is drawn overhead along with light hydrocarbons through line 23 and cooler 24 to HF settler 25 which is preferably operated at a temperature obtainable with ordinary condenser water. Any condensed hydrocarbons separate out as an upper layer and they may flow over baffle 26 and be withdrawn through line 27. A portion of such material may be employed as a stripping gas in stripper 21 and/or in the complex stripper which will be hereinafter described. The net production of the condensed hydrocarbons may be passed through a bauxite tower or otherwise treated to remove HF and/or combined fluorides. Similarly the gas vented from the settler through line 28 may be freed of HF and utilized in any conventional manner. The acid layer is withdrawn through line 29 to HF storage tank 30 from which it is supplied to line 13 by pump 31.

The stripped saturated oil leaves the base of stripper 21 through line 32 and is then fractionated in a conventional system diagrammatically illustrated by tower 33, the light hydrocarbons such as gasoline being taken overhead through line 34 and the heavier hydrocarbons being withdrawn through line 35.

The HF phase which may in this case consist of about 10 to 20 weight percent of unsaturated hydrocarbon material and 80 to 90% by weight hydrogen fluoride is withdrawn through line 36 to HF-complex stripper 37 to which a stripping gas (e. g. from line 27) may be introduced through line 38. Heating means 39 may be employed at the base of this stripper but the temperature thereof should not exceed about 300° F. and preferably should be not higher than about 150° F. to 200° F. in order to avoid degradation of the HF-hydrocarbon complex. The stripping in tower 37 should be sufficient to remove the uncombined HF but to leave at least 1 molecule and preferably 1½ to 2 molecules HF per double bond of olefinic material contained in the HF solution. In other words, the HF content of the introduced mixture should be reduced to about 35 to 50% by weight but should not be reduced to less than about 30% by weight.

The HF and stripping gas which leaves the top of stripper 37 through line 40 may be combined with the overhead from stripper 21; a part of the overhead may be introduced through branched line 41 into the upper part of stripper 21 and another part may be introduced directly to line 23.

The HF-unsaturated oil complex from the base of stripper 37 is introduced through cooler 42 and line 43 into a hydrolyzing system 44 which is shown as a continuous countercurrent tower in Figure 1 and as a multiple batch system in Figure 2. Hydrolysis is effected by means of an aqueous HF solution containing at least about 1 part HF to 2 parts water, said solution being introduced through line 45. The amount of HF solution introduced is controlled so that the final HF : water

ratio in the aqueous HF solution leaving by line 51 will be in the range of 1:1 (i. e. 50 weight percent HF) to 4:1 (i. e. 80 weight percent HF) if viscous products are desired; if non-viscous fluid oils are desired, the final HF : water ratio should be less than 1:1. In the system diagrammatically illustrated in Figure 1, hydrolysis is effected in a countercurrent tower which may be provided with suitable mixers or contacting surfaces and which may be provided with a series of cooling coils 46, 47 and 48 for temperature control. At the complex inlet end the temperature should be relatively low, e. g. about 35 to 85° F. At the upper end of the hydrolyzing tower where the complex has been substantially denuded of combined HF, a higher hydrolyzing temperature of the order of 125 to 175° F. may be employed for removing as much as possible of the combined HF and to decrease the viscosity of the polyolefinic oil so as to facilitate the separation of oil and aqueous phases. When producing extremely viscous oil, it is advantageous to introduce a light hydrocarbon diluent stream, such as pentane, into tower 44 in order to facilitate the separation of the desired polyolefinic oil. While the use of a countercurrent system with a temperature gradient as hereinabove described is preferred, it should be understood that the hydrolysis may be effected at a substantially constant temperature attainable by cooling water or refrigeration, i. e. in the range of 35 to 125° F. or about 60° F.

For obtaining a "fractionation" of the polyolefinic oil components (i. e., a separation of the oil into components of higher and lower degrees of unsaturation and improved color) in the hydrolyzing step it may be desirable to employ one or more stirred batch-type hydrolyzers as illustrated in Figure 2. This may be accomplished by a step-wise addition of the hydrolyzing medium. Complex from line 43 and aqueous HF (approximately 1.6 parts water and 1 part HF) from line 45 are introduced into stirred mixing vessel 44a which is provided with a jacketed cooler 48a. The amount of aqueous HF may be regulated to produce a concentrated HF layer containing about 3-6 parts of HF per part of water by weight. After intimate mixing for a period of 2 to 20 minutes at about 35 to 150° F., an equal volume of pentane or other light hydrocarbon diluent is added and the mixture stirred for 5-10 minutes additional. The mixture is then introduced by line 49 into batch settler 50. After settling for about 20 minutes the concentrated aqueous HF solution is withdrawn from settler 50 through line 43a where it is mixed with an additional quantity of aqueous HF from line 45b. A pentane solution of an oil "A," of comparatively low iodine number (e. g. about 250), is then removed through line 51a amounting to about 10-20% of total oil contained in the complex. Oil "A" is finally recovered from the pentane solution by any conventional stripping method; color of the recovered oil "A" is about 5 ASTM. The concentrated HF solution previously removed from settler 50 and mixed with additional aqueous HF from line 45b is then introduced into mixing vessel 44b. After stirring for another 2 to 20 minutes in this mixer while maintaining a temperature of 35 to 150° F., by cooling jacket 47b, an equal volume of pentane is added and stirred as described above. The mixture may then be introduced by line 49' into settler 50' from which aqueous HF is withdrawn through line 51b and a pentane solution of crude higher iodine number drying oil "B" is with-

drawn through line 52. The aqueous layer withdrawn from settler 50' should contain at least about 1 part of HF per part of water by weight and may for example contain 1.2-1.8 parts of HF per part of water. Depending on the final aqueous HF concentration, 75-90% of the remaining oil will be recovered in the second hydrolyzing step; this oil has a color of 6-8 ASTM. The aqueous layer withdrawn from line 51b may be subjected to a third hydrolyzing operation or it may be sent to an HF distillation tower wherein HF is recovered.

Regardless of the particular type of hydrolysis system employed, the crude drying oil solution which leaves said system through line 52 will still contain a small amount of HF which is usually less than .3% and is preferably less than .1%. To remove final traces of HF the crude drying oil solution may be contacted with bauxite but it is preferably neutralized with ammonia, lime slurry or a concentrated caustic solution introduced through line 53 and intimately mixed with the crude drying oil solution in mixer 54. The mixture then passes to settler 55 from which the caustic is settled out and withdrawn through line 56, most of the caustic being recycled by pump 57 and a very small amount of spent caustic being withdrawn through line 58.

The neutralized product may then be distilled under subatmospheric pressure after preliminary distillation for removal of pentane (preferably in the range of 1 to 10 mm.) in conventional distillation equipment illustrated by tower 60, the gasoline boiling range materials being taken overhead through line 61, drying oil distillate being recovered through line 62 and a high boiling polyolefinic drying oil or resin being withdrawn through line 63. Fractions of any desired boiling ranges may thus be obtained. Atmospheric flash distillation may be employed where the time at elevated temperatures is minimized. A preferred operation is atmospheric distillation in a first tower to remove the solvent and the lowest boiling component followed by vacuum distillation in a second tower for separation of one or more drying oil fractions.

The aqueous liquid withdrawn from the hydrolyzing system may contain about 40 to 80%, usually about 45 to 65% by weight of HF, and such solution is withdrawn by line 51 (or 51a and 51b) and introduced into HF fractionator 64 which is provided with a suitable heater 65 at its base and reflux coil 65a at the top. This fractionator is carefully operated to distill overhead substantially anhydrous HF from a constant boiling mixture of about 1 part HF and about 1.6 parts water. At atmospheric pressure such distillation may be effected at a temperature of about 70° F. at the top of the tower and about 230° F. at the bottom of the tower. The anhydrous HF passes through line 66 and condenser 67 to HF storage tank 30 at 20 pounds pressure, the temperature at the top of the tower will be about 110° F. with about 275° F. at the bottom. The constant boiling mixture, which may be about 1 part HF and 1.6 parts water but which will vary slightly in composition depending on the pressure in tower 64, is returned by pump 68 and line 45 to the hydrolyzing system. Some oil may be associated with the constant boiling mixture from tower 64 and should be separated by decantation in a suitable settler.

In starting up the operation, the hydrolysis is effected by introducing water from line 69 into line 45 but once the required amount of water is introduced, it simply circulates around and

around between hydrolyzer 44 and HF fractionator 64, the water removing HF from the complex in the hydrolyzer and HF being removed from the water in the HF fractionator. If any additional water enters the system it will tend to build up in this cycle in which case dilute HF must be removed through line 70. Since the recovery of HF from such a dilute solution is a difficult and expensive procedure it is important to avoid any such build-up and to employ charge materials which are substantially anhydrous. Generally speaking, the solution introduced from the HF fractionator to the hydrolyzer should contain about 36 to 40% HF and the solution returned from the hydrolyzer to the stripper should contain about 45 to 65% HF. It may however be possible to alter the amount of HF in the solution by employing water soluble additives such as HF salts.

From the description it will be seen that the objects of the invention have been attained. The invention is not limited, however, to the details hereinabove set forth since many modifications of equipment and alternative procedures, conditions and proportions will be apparent from the above description to those skilled in the art.

We claim:

1. The method of hydrolyzing an HF-polyolefinic hydrocarbon complex wherein the polyolefinic hydrocarbon component contains about 4 to 6 double bonds per molecule which method comprises initially contacting said complex with an aqueous HF solution containing at least about 50 but less than 80 weight percent HF while removing heat of hydrolysis and effecting said hydrolysis by initially contacting the complex with a portion of said solution at a temperature below about 85° F. and contacting partially hydrolyzed complex with a portion of said solution at a higher temperature which is below 200° F.
2. The method of obtaining a viscous high molecular weight drying oil having a high iodine number from an HF-hydrocarbon complex obtained by treating a hydrocarbon oil which is substantially free from aromatic hydrocarbons with hydrogen fluoride at a conversion temperature not higher than 450° F. with an HF to oil ratio in the range of .2:1 to 5:1 and for a contact time sufficient to obtain substantial conversion followed by separation of an HF phase containing said complex dissolved in a large amount of free HF from a saturated oil phase containing a small amount of dissolved HF, which method comprises stripping said HF phase at a temperature in the range of about 100° to 250° F. under conditions for removing substantially all free HF and for leaving complex which contains about 1 to 2 molecules of HF per double bond of the hydrocarbon component of the complex, hydrolyzing with an aqueous HF solution said complex which contains at least 30 weight per cent combined HF but not more than 50 weight per cent HF after the removal of free HF therefrom, initially contacting said complex in the hydrolyzing step with an aqueous HF solution said complex which contains at least about 50 but less than 80 weight per cent HF, effecting at least the initial part of hydrolysis at a temperature in the range of 35° to 125° F. and effecting all of the hydrolysis at a temperature below 200° F., separating aqueous HF from hydrolyzed complex, removing residual HF from said hydrolyzed complex to obtain HF-free hydrocarbons and distilling said HF-free hydrocarbons at subatmospheric pressure.
3. The method of claim 2 which includes the

15

additional step of increasing the temperature of the complex-aqueous HF mixture after initial hydrolysis to a temperature in the range of 125 to 175° F.

4. The method of claim 2 which includes the step of adding a sufficiently small amount of aqueous HF so that the amount of HF in the aqueous HF composition after hydrolysis will be in the range of 55 to 65 weight per cent. 5

5. The method of claim 2 wherein the hydrolyzing is accomplished by stepwise addition of said aqueous HF solution and wherein a light hydrocarbon diluent is added to the hydrolyzed mixture to facilitate phase separation. 10

ROBERT J. LEE. 15  
PAUL D. MAY.

16

## REFERENCES CITED

The following references are of record in the file of this patent:

## UNITED STATES PATENTS

| Number    | Name      | Date          |
|-----------|-----------|---------------|
| 2,436,695 | Kuhn      | Feb. 24, 1948 |
| 2,440,459 | Bloch     | Apr. 27, 1948 |
| 2,470,894 | Johnstone | May 24, 1949  |